

(No Model.)

C. KUHL.

FLAG STONE AND CEMENT PAVEMENT.

No. 406,289.

Patented July 2, 1889.

FIG.1.



FIG.2.



FIG.3.



Witnesses

Frank L. Willard.  
W. G. Murray

Inventor

Charles Kuhl  
By his Attorney Geo. J. Murray

# UNITED STATES PATENT OFFICE.

CHARLES KUHL, OF CINCINNATI, OHIO.

## FLAG-STONE AND CEMENT PAVEMENT.

SPECIFICATION forming part of Letters Patent No. 406,289, dated July 2, 1889.

Application filed February 16, 1889. Serial No. 300,101. (No model.)

*To all whom it may concern:*

Be it known that I, CHARLES KUHL, a citizen of the United States, and a resident of Cincinnati, in the county of Hamilton and State 5 of Ohio, have invented certain new and useful Improvements in Flag-Stone and Cement Pavements, of which the following is a specification.

In localities where freestone is readily obtained it has been extensively used as a paving-stone, because it is easily dressed and does not become slippery from wear; but when used on much-traveled thoroughfares wears unevenly, so that it becomes necessary to take 15 up the stones, dress them, and again reset them. This is a troublesome and expensive operation, and in many cases the stones are worn so thin as to render it impracticable.

The principal object of my invention is an 20 economical means to repair these pavements without removing the stones from place.

Another object of my invention is to provide the common limestone, sandstone, or granite pavements with a good walking-surface, and thus avoid the expense of dressing 25 the stones off even and prevent the pavement from becoming slippery in wet weather.

I will first describe my invention in connection with the accompanying drawings, 30 after which it will be particularly pointed out in the claims.

Figure 1 is a vertical transverse section of a pavement repaired according to my invention. Fig. 2 is a similar section of the pavement before repairing. Fig. 3 is a vertical longitudinal section through line  $xx$  of Fig. 1.

The stones A, as seen in Fig. 2, are first chipped down roughly even with or a little below the lowest worn part, as seen in Figs. 40 1 and 3. A thin binding-coat B, composed of clean fine sand and Portland cement in about equal parts, is then floated over them. After this becomes set I prepare a concrete C, of coarse gravel or finely-broken stone, fine sand, 45 and Portland cement, about two parts of the gravel or broken stone well mixed with a mortar composed of two parts of sand and one part of Portland cement. This is put on to the thickness of about one inch and a half 50 to two inches and tamped down firmly. Then

an upper finishing coat D, of fine sand and Portland cement in about equal parts, is floated on to the depth of three-fourths of an inch to an inch, and while the material is still in a plastic state it is severed with a trowel 55 through to the joints between the stones, and the joints so made finished with a marker, thus giving the pavement its original appearance. The separation of the concrete permits it to shrink in setting without cracking 60 irregularly.

In many parts of the country limestone flagging is extensively used for sidewalks. These stones are found in regular layers of from three to six inches in thickness, and are 65 commonly used without dressing, partly to save the labor, but principally because if dressed they soon wear smooth and are very slippery in rainy weather. In their rough or unfinished state these stones soon weary the 70 feet, especially of persons who wear thin-soled shoes. I find that the finishing coat I have above described, of sand and Portland cement, adheres very firmly to these flag-stones, especially when first taken from the quarry and 75 thoroughly cleaned. After the paving-stones are placed in position I coat their upper surface with this concrete to the thickness of about an inch, then divide the concrete in the same line as the joints between the stones, 80 and finish the joints in the usual manner. When these stone pavements have been used so long that the stones have worn smooth, the surface should be first roughened or bush-hammered before applying the coating-surface 85 in order to cause it to adhere firmly.

I find from experience that the proportions I have above given for forming the concretes are the best; but they may be varied without a departure from my invention, and it is also 90 evident that the coarse concrete C may be omitted from the first-described pavement and the fine concrete alone used; but in the latter case the pavement would be no better and would cost much more to repair it. 95

What I claim as new, and desire to secure by Letters Patent, is—

1. The combination, in a pavement, of the stones roughened upon the upper surface, the binding-coat B, placed on the same, the coarse 100

concrete C, and the finishing coat D, the whole arranged and the block divided, substantially as specified.

2. The method herein described of repairing stone pavements, which consists of the following steps: first, cutting down and roughening the uneven surfaces of the stones; second, coating the upper surface with a binding-coat of cement and sand; third, placing on

the same a concrete coating composed of coarse stone, sand, and Portland cement; fourth, placing upon the coarse concrete a finishing coat of fine sand and Portland cement, substantially as specified.

CHAS. KUHL.

Witnesses:

BEN B. DALE,  
M. L. MURRAY.